

## UNITED STATES PATENT OFFICE

1,959,087

METALLIC FOIL AND METHOD OF  
MANUFACTURE

Urlyn Clifton Tainton, St. Louis, and Frank W. Harris, Clayton, Mo.; said Harris assignor to said Tainton

No Drawing. Application April 20, 1931,  
Serial No. 531,610

8 Claims. (Cl. 29—18)

This invention relates to metallic foil, and with regard to certain more specific features, to improved methods of producing metallic foil having smooth bright surfaces.

5 Among the several objects of the invention may be noted the provision of metal for manufacturing foil which may be processed to secure foil having a desirable, bright surface; and the provision of a process for economically manufacturing thin metal foil having a smooth bright surface. Other objects will be in part obvious and in part pointed out hereinafter.

The invention accordingly comprises the elements and combinations of elements, steps and sequence of steps and features of synthesis which will be exemplified in the description hereinafter and the scope of the application of which will be indicated in the following claims.

Metal foil is manufactured from the less precious metals by subjecting a strip of metal to repeated rolling operations until the thickness is reduced to the desired degree. The unit cost of this rolling operation is greatly reduced by a procedure known as pack-rolling, comprising placing a number of strips of metal together and passing them simultaneously through rolls. This latter method, however, is objectionable in that the foil produced thereby, except for the two outside surfaces of the outer pieces in contact

30 with the rolls, has a "matte" or "eggshell" surface instead of the smooth bright surface which is desired. It has not been possible hitherto to produce a smooth bright surface on foil except by actual contact with a polished roll. This fact

35 has operated to the advantage of metals such as lead and tin which on account of their softness can be readily rolled at high speeds and easily take a bright finish from the rolled surface. It has operated to the disadvantage of other metals,

40 and in particular of zinc. Although intrinsically cheaper than lead and tin per unit of foil produced, by present methods zinc cannot be given a bright surface except by a relatively expensive operation of individual piece rolling with polished

45 rolls. For this reason the majority of the foil produced has been made from the relatively expensive lead and tin or a combination of these. Zinc, on account of its greater strength and lower specific gravity, can be made to give three times

50 as many square inches of foil per pound of original metal as can the lead-tin combination generally used.

It has hitherto been supposed that the production of a dull surface on the inside sheets of

a crystalline or non-homogeneous structure and do not resist deformation of the surface equally at all points. Accordingly when two metal surfaces are pressed together under exterior force, the harder parts of one metal project into the softer parts of the other and thus produce a rough or dull, "eggshell" or "matte" surface on each.

Although this dull effect has been thought to be characteristic of all metals, we have discovered that in the case of zinc it can be prevented. Zinc possesses to a high degree a property which may be termed plasticity or ductility, that is to say, zinc has characteristics such that even when cold it will yield or flow gradually under applied stress. This property is undesirable for most structural purposes and considerable work has been done in the direction of alloying zinc with other metals in order to overcome this plasticity. A common example of a zinc alloy in which the plasticity or ductility has purposely been destroyed is die casting metal, which normally consists of 93% of zinc and 7% of copper, aluminum and magnesium. This die casting alloy is hard and strong and does not flow under stress. Other alloys have been developed to improve the qualities of zinc as a structural material for roofing sheets, piping, etc.

For the purposes of this invention, however, it is desirable that the plastic or ductile properties of the zinc metal be retained. It is also desirable to restrain or prevent the recrystallization which occurs in pure zinc even at ordinary or room temperatures, which itself occasions a matte surface when zinc sheets are rolled in a pack.

We have discovered that certain substances if added to the zinc in proper amount will inhibit this recrystallization property while not substantially decreasing, and in some cases actually increasing, the plastic or ductile properties of the metal. It is important that the added substances be not present in such amounts as to produce a hard strong metal, which while useful for ordinary purposes, would be of little utility for the purposes herein considered. For example, any substantial amounts of iron, cadmium or magnesium would be detrimental to the purposes of this invention.

Our researches have shown that the desired effect may be produced by the addition to pure zinc of various elements in carefully graduated amounts. In the case of metals which form a brittle eutectic alloy with zinc, the amount of alloying metal added should be less than is required to form the eutectic. If aluminum be

75

65

70

75

85

90

95

100

105

110

used, for example, the amount added should be less than 5.0%, this representing the corresponding eutectic mixtures. The following metals have been tried and found effective for our purposes:

5 Antimony in amounts up to 4%.

Copper and aluminum in amounts up to 2%.

Tin and silver in amounts up to 1%.

Mercury in amounts up to 1%.

10 Various combinations of these metals have proved effective and it is probable that other metals may also be used. On account of the large number of the elements, it is not possible to cover in this specification all of the combinations of zinc with other metals that may be effective. Accordingly we do not wish to limit ourselves to the metals specified but may use any substances which when added to zinc metal will restrain or even totally inhibit the recrystallization 15 of the metal, which normally occurs at ordinary temperatures, and at the same time will not substantially diminish the plasticity or ductility of the metal.

It is not necessary for the purpose of this invention that the added substances be metals. We have also found that pure zinc electrolytically deposited from a solution containing colloids occludes sufficient of the colloid to prevent recrystallization of the zinc and thus may be used 25 according to this specification with the production of bright foil surfaces throughout the pack.

As an illustration of the method of carrying this invention into effect we will describe the production of bright foil from cathode zinc and 30 also from an alloy. In the former case, according to our preferred method, zinc is deposited from a sulphate solution containing about 250 grams per liter of sulphuric acid and about 60 grams per liter of zinc at a cathodic current density of about 100 amperes per square foot. To the electrolyte is added a colloid such as 35 silicic acid or gum arabic in amounts representing about one to four pounds per ton of zinc deposited.

40 The zinc may be deposited upon a starting sheet of aluminum from which it may be readily detached when it has reached the required thickness. Alternatively, the zinc deposit may be built upon a thin starting sheet of zinc which when 45 completed can be rolled without separation of the deposit from the starting sheet. In the production of continuous strips of foil a drum-shaped aluminum cathode surface may be employed, this being rotated at the appropriate speed according to known methods so that a 50 continuous strip of cathode zinc is produced which after washing with water may be passed directly to the rolls. After a zinc cathode has been given a preliminary rolling operation, several sheets are superimposed and passed through the rolls as a pack. We have successfully 55 rolled as many as thirty-two sheets at a time in this way. Preferably, the roll should be conducted at ordinary temperatures, as increasing 60 temperature tends to promote recrystallization of the zinc. It is also of advantage to separate the sheets occasionally during the rolling operation, though not necessarily after each passage 65 through the rolls.

70 It will be found that foil made in this way can be rolled to a thickness of .0003 inch or less, which represents a yield of about 13,500 square inches per pound of zinc. All of the foil so produced will be found to have a bright surface even 75 though it may have been reduced to one-hun-

dredth of its original thickness without contact with the roll surfaces.

To produce a corresponding foil in the case of an alloy we prefer to start with the highest grade zinc commercially available, with an analysis of 99.99% pure or higher. This is melted and while in the molten state the appropriate amount of other metal is introduced. In a typical case for example we add to one ton of molten zinc say three pounds of copper and one pound of antimony. The metal is thoroughly mixed and then poured into a mold to form a slab, for example, two inches thick and of dimensions appropriate to the length and width of strip desired. The first rolling is carried out at an elevated temperature, say 250° C. When the thickness has been suitably reduced, say to one-thirtieth of an inch, the strip is cooled down and then pack-rolled as described above in the case of the cathode deposited zinc. This procedure also will be found to result in a foil with a brilliant, shining surface although this surface is not derived from contact with the rolls themselves.

80 Summarizing the foregoing, it will be seen that our invention offers the following advantages:

85 1. A much greater area of foil can be obtained from a given weight of the modified zinc herein described than from the lead-tin combination normally used. On account of the relatively low cost of zinc this permits a great saving in cost.

90 2. The foil produced is of exceptionally good quality and pleasing in appearance. The surface retains its brightness when exposed to oxidation, dirt, fingermarks, etc., much longer than in the case of foil having a dull surface. Moreover, the zinc foil is considerably stronger and tougher than the lead-tin foil which is now ordinarily used and will therefore withstand more handling and bending without breakage.

95 3. On account of the fact that a large number of strips can be rolled simultaneously, the production capacity of a set of rolls is much greater than when rolling single or double sheets, and rolling costs are correspondingly reduced.

100 In view of the foregoing, it will be seen that the several objects of the invention are achieved and other advantageous results attained.

105 As many changes could be made in carrying out the above compositions and procedures without departing from the scope of the invention, it is intended that all matter contained in the above description shall be interpreted as illustrative and not in a limiting sense.

110 We claim:

115 1. The process of producing metallic foil having a smooth bright surface from zinc, said process comprising alloying at least one second metal with said zinc, said second metal being of a character and sufficient in amount to restrain said zinc from re-crystallization at ordinary temperatures when worked cold by compressive operations but only in such amount as will leave the resulting metal produce ductile and workable cold by compressive operations, and then simultaneously cold rolling a number of sheets formed from said alloy superimposed upon one another.

120 2. The process of producing metallic foil having a smooth bright surface from zinc, said process comprising alloying copper and antimony, with said zinc as the basic material, in percentages to inhibit recrystallization when the resulting zinc alloy is worked cold by compressive operations, said copper and antimony being employed in such amounts that while re-

125

130

135

140

145

150

155

160

165

170

175

180

185

190

195

200

- straining or inhibiting the re-crystallization of said zinc at ordinary temperatures they are not employed in sufficient amount to destroy the ductility and cold workable characteristics of 5 the basic zinc material, and then simultaneously cold rolling in superposed relationship a number of sheets formed from said alloy. 3. The process of producing a metallic foil having a smooth bright surface from substantially pure zinc, said process comprising electrolytically depositing said zinc from a solution having therein a colloid, said colloid inhibiting re-crystallization of said zinc at ordinary temperatures but of a character to leave the resulting zinc product with its ductile characteristics, and simultaneously rolling a number of sheets formed from said electrolytically deposited zinc superimposed upon one another to form said metallic foil. 4. The process of producing metallic foil having a smooth bright surface from substantially pure zinc, said process comprising electrolytically depositing said zinc from a solution having therein gum arabic, said gum arabic inhibiting re-crystallization of said zinc at ordinary temperatures but leaving the zinc product with relatively ductile characteristics that lend to cold working by successive compressive operations, and simultaneously cold rolling when superposed one upon another a number of sheets formed from said electrolytically deposited zinc to form said metallic foil. 5. A rolled metallic foil having a smooth bright surface and composed of zinc containing a substance capable of restraining or inhibiting the recrystallization characteristic of pure zinc at ordinary temperatures. 6. A rolled metal foil as per claim 5, in which an occluded colloid is relied upon to provide a material whereby the recrystallization characteristic is inhibited. 7. A rolled metal foil as per claim 5, in which at least one second metal is relied upon for preventing the recrystallization characteristic of zinc during the rolling process. 8. A rolled metal foil as per claim 5, in which at least one second metal, as copper or antimony, is relied upon for restraining the recrystallization characteristic of zinc during the period while the rolling into the form of a foil is taking place.
- 30 100  
URLYN CLIFTON TAINTON.  
FRANK W. HARRIS.
- 35 110
- 40 115
- 45 120
- 50 125
- 55 130
- 60 135
- 65 140
- 70 145
- 75 150